

## UNITED STATES PATENT OFFICE.

HARRY A. GRINE, OF CLARKSBURG, WEST VIRGINIA, ASSIGNOR TO THE GRASSELLI CHEMICAL COMPANY, OF CLEVELAND, OHIO, A CORPORATION OF OHIO.

## ZINC CONDENSER.

No Drawing.

Application filed April 3, 1924. Serial No. 703,979.

To all whom it may concern:

Be it known that I, HARRY A. GRINE, a citizen of the United States, and a resident of Clarksburg, county of Harrison, and 5 State of West Virginia, have invented a new and useful Improvement in Zinc Condensers, of which the following is a specification, the principle of the invention being herein explained and the best mode in which 10 I have contemplated applying that principle, so as to distinguish it from other inventions.

The present invention, relating, as indicated, to zinc condensers, is more particularly directed to an improved condenser for use in the retort or muffle smelting of oxidized zinc ores to produce metallic zinc, the principal object of the invention being the provision of a condenser of this type and 20 purpose which shall have a high content of zinc-bearing material and low clay content. A further object of the invention is the provision of such a condenser which shall have a greater heat conductivity, greater condensing efficiency, and shall be capable of 25 re-use when broken up, with a minimum of low zinc-bearing materials in the broken condenser product which is to be re-charged. Other objects of the invention will appear 30 hereinafter. To the accomplishment of the foregoing and related ends, said invention, then, consists of the means hereinafter fully described and particularly pointed out in the claims, the following description setting 35 forth in detail one method and one product exemplifying my invention, such disclosed procedure and product constituting, however, but one of various applications to the principles of my invention.

40 The present practice of retort or muffle smelting of oxidized zinc ores to produce metallic zinc involves the introduction of the zinc ores and reducing fuel into a retort or muffle which is mounted in a furnace 45 chamber in which the temperature is maintained at the proper heat for reduction of the ore. Condensers are set in the mouth or open end of the muffles of retorts and luted thereto with finely-ground anthracite culm 50 which forms a joint between retort and condenser which is impervious to zinc vapors under the low pressure within the retorts. These condensers project without the furnace chamber and cause sufficient drop in 55 temperature of the zinc vapors issuing from

the retorts to condense them and also serve to retain the metal after condensation until drawn. The present condensers consist in composition of about nine parts by volume of burned clay or grog to seven parts of raw 60 plastic refractory clay. Neither of these materials contain zinc in smeltable quantity, only a very small per cent being contained in reclaimed retort or condenser material used as grog in the making of new 65 condensers. The burned clay may be either new material used for the first time, or it may be all or partly burned clay material recovered from broken retorts or condensers 70 which have been used.

At the end of each day's operations the condensers are removed from the mouth of the retorts or muffles to allow the removal of the residues from the muffles, after which the retorts are charged with new ore and fuel. In removal a number of the condensers are broken, and certain condensers are discarded because of the accumulation 75 of zinc oxide, zinc dust or blue powder and metallic zinc on the inside of the condenser, which material has a higher melting point than the metallic zinc and gradually covers the condenser with a coating up to one inch in thickness. The broken and discarded 80 condensers are broken up and the condenser man selects the portions with the heaviest 85 deposits of zinc thereon, these selected portions being broken into small pieces and then recharged into the furnace along with the new ore and fuel. In this way a certain amount of the deposits on the condensers 90 are saved for the recovery of zinc contained.

My improved condenser is formed of a composition which is high in zinc bearing materials and relatively low in refractory clay and other low or non-zinc-bearing materials, which allows the condensers after use to be completely broken up and recharged, with a saving of practically all of the residues on the condenser and of the zinc content in the condenser itself. My improved condenser may be formed of a mixture containing approximately 80 per cent to 85 per cent of zinc-bearing material, assaying 25 per cent or more zinc, such for example as 95 broken used ore condensers, calcined Joplin ore, which contains about 68 per cent zinc and a small amount of finely pulverized plastic clay as a bonding material. I use 100 these materials in the proportions of about 105

- 45% of the broken used ore condenser, 45% of new ore and 10% of plastic bonding clay. A condenser mixture formed of these materials will have approximately 52% or 5 53% zinc content before use and a zinc content after use for seven or eight days of about 65%. Various bonding materials may be used, such, for example, as fire clays or bentonite, and these and others have been 10 found entirely suitable for this purpose.

After condensers of my composition are discarded they are broken up to pass a four-mesh screen, and this crushed material is then mixed with ore and charged into the 15 furnace, thus returning to the furnace all of the zinc material.

In making my condensers I may use some of the discarded condenser material crushed to pass a four-mesh screen, which is then 20 thoroughly mixed with calcined zinc ore or zinc ash, or materials of a similar nature, which has been crushed to pass a 20-mesh screen, or may use straight zinc ore, and then mixed with plastic clay or other bonding materials, which have been crushed to 25 pass a 40 to 60-mesh screen. These various materials are then pugged through a wet mixing pug mill in the usual manner and allowed to stand for several days and then 30 re-pugged, after which the material may be molded into condensers in the machine commonly used for this purpose. After molding the condensers are placed in a drying room and baked at a temperature of 35 from 100° to 140° F. for 10 to 15 days, and then given a second baking at a higher temperature of from 150° to 175° F. before use.

My condensers have a higher strength than 40 those now in use, and in this way effect a considerable saving, as less are broken in handling. They also have a greater heat conductivity since the walls may be thinner because of the greater strength of the material. In addition, these condensers have 45 a higher condensing efficiency because of the greater heat conductivity of the material and the thinner walls of the condenser. The use of thinner walls effects a saving in the 50 breaking up of the condensers after use for

subsequent recharging and also in concentrating costs where wet concentration or hand chipping and selection of condensers is practiced.

In addition to the above advantages I effect a considerable saving in zinc, which is in present practice lost because of pieces of condenser discarded and not recharged, and a greater efficiency in the furnacing operation because of the absence of considerable 55 amounts of refractory materials which are unavoidably included with the zinc from the broken-up condensers under the present practice and availability of the retort capacity, which would be occupied by such 60 barren material, for the smelting of zinc-bearing material.

Other forms may be employed embodying the features of my invention instead of the one here explained, change being made 70 in the form or construction, provided the elements stated by any of the following claims or the equivalent of such stated elements be employed, whether produced by my preferred method or by others embodying steps equivalent to those stated in the 75 following claims.

I therefore particularly point out and distinctly claim as my invention:—

1. A composition for zinc condensers comprising broken zinc condenser, zinc ore and a refractory bonding material.

2. A composition for zinc condensers comprising approximately 80 per cent zinc-bearing material consisting of equal parts 85 of broken zinc condenser and zinc ore and 20 per cent refractory bonding material.

3. A composition for zinc condensers comprising equal parts of broken zinc condenser and zinc ore, each having a zinc content in 90 excess of 60% and a small amount of plastic refractory clay.

4. A composition for zinc condensers comprising equal parts of broken zinc condenser and zinc ore, each having a zinc content in 95 excess of 60%, and about 10% of plastic refractory clay.

Signed by me, this 24 day of March, 1924.

HARRY A. GRINE.